

## UNITED STATES PATENT OFFICE

2,183,009

## LUBRICATING OIL

Joseph Cole, Whiting, Ind., assignor to Sinclair  
Refining Company, New York, N. Y., a corpora-  
tion of Maine

No Drawing. Application September 23, 1936,  
Serial No. 102,167

4 Claims. (Cl. 37—9)

My invention relates to improvements in pour  
depressors, compounding agents to be added to  
petroleum lubricating oils to lower the tempera-  
ture at which such oils cease to flow, and in  
methods of making such pour depressors.

5 I produce the pour depressor of this invention  
by mixing stearic acid with chlorinated paraffin  
wax and treating this mixture with anhydrous  
aluminum chloride.

10 Specifically, the pour depressor of this invention  
is conveniently produced as follows: A mixture  
of 200 parts (by weight) of chlorinated  
paraffin wax containing about 43% (by weight)  
of chlorine and 100 parts of stearic acid is heated  
15 to 120° F. and maintained at that temperature  
for 30 minutes. 15 parts of anhydrous aluminum  
chloride is added to the resulting mixture, and  
the temperature of this mixture is gradually in-  
creased, while maintaining thorough stirring,  
20 until a temperature of 580° F. is attained. The  
mixture may then be filtered while still hot. The  
product of this aluminum chloride treatment is  
the pour depressor of my invention. It remains  
liquid at room temperature.

25 This pour depressor may be compounded with  
petroleum lubricating oils in proportions rang-  
ing from a fraction of a percent up to several  
percent, from 0.1% to 1% or somewhat more  
for example. Added to one Pennsylvania lubri-  
cating oil originally having a pour test of 25° F.,  
30 0.5% (on the oil) of this pour depressor pro-  
duced a compounded product having a pour test

of —15° F. Such reductions in the pour test  
are attained without impairment of the viscosity  
index of the oil, but the compounded products  
are usually darker in color than the oil before  
addition of the pour depressor.

My invention includes this pour depressor and  
petroleum lubricating oils compounded with this  
pour depressor as well as the method of mak-  
ing the pour depressor. However, I do not now  
have any better mode of identification of the 10  
pour depressor than the method by which it is  
made.

I claim:

1. A method of making a pour depressor com-  
prising reacting chlorinated paraffin wax with 15  
stearic acid in the presence of anhydrous alu-  
minum chloride, and removing the solid con-  
stituents from the liquid product of this reaction.

2. A pour depressor which comprises the prod-  
uct produced as in claim 1.

3. Compounded petroleum lubricating oils com-  
prising the pour depressor produced as in claim 1.

4. The method of depressing the pour point of  
a petroleum lubricating oil which comprises re-  
acting chlorinated paraffin wax with stearic acid 25  
in the presence of anhydrous aluminum chloride,  
to form a liquid product, removing solid con-  
stituents from this liquid product, and adding  
the liquid product to the petroleum lubricating  
oil.

JOSEPH COLE.